

Jan. 1, 1935.

B. BANNISTER

1,986,704

PROTECTIVE COATING FOR METALS

Original Filed June 11, 1932



Fig. 1.



Fig. 2.



Fig. 3.

Inventor:  
BRYANT BANNISTER,  
by: *Maurice Lauber*  
his Attorneys.

## UNITED STATES PATENT OFFICE

1,986,704

## PROTECTIVE COATING FOR METALS

Bryant Bannister, Mount Lebanon, Pa.

Continuation of application Serial No. 616,609,  
June 11, 1932. This application March 14,  
1933, Serial No. 660,720

## 6 Claims. (Cl. 148—7)

This invention relates to protective coatings for metal articles and particularly for metal piping, and is a continuation of my co-pending application, bearing the same title, Serial No. 5 616,609, filed June 11, 1932.

An object of the invention is to produce a new and improved method of applying a coating of protective material to the surface of an article.

A further object is to produce a new and improved method of forming a protective alloy coating on the surface of a metal article such as a pipe or conduit.

The general use of pipe lines for transporting gas, oil and such liquids over long distances, has accentuated the necessity for providing cheap piping, which is durable under varying atmospheric and soil conditions. The question of expense renders the use of non-corrosive metals in the manufacture of pipe for such purposes prohibitive, with the result that the art has necessarily turned to ferrous metals, and various attempts have been made to solve the problem of external corrosion. If assured of corrosion protection, the wall thickness of the pipe could be reduced to that necessary for mechanical strength, since extra metal would then not be necessary to provide for the expected loss of strength resulting from corrosion. With this in mind, it is apparent that the resultant saving in material and the elimination of costly maintenance would amply justify incurring considerable expense in providing a corrosion-free pipe.

As stated, the problem of protecting steel or iron piping against external corrosion has been the subject of considerable research within recent years but, up to the present time, the various methods and procedures advocated have only been partially effective. This is primarily due to the fact that it has been impossible to so coat iron or steel surfaces with a protective covering as to avoid scaling or checking of the covering or the presence of minute pin holes in the covering. The result of either is detrimental, since the possibility for corrosion is not eliminated and after corrosion starts it is apt to progress quite rapidly, with the result that the base and the protective surface are damaged and a condition is promoted which favors the progress of the corrosion.

One of the more specific objects of my invention is to produce a thin but impervious protective alloy on the surface of a metal base. It is apparent that the ideal pipe for corrosion resistance, would be composed entirely of corrosion resistant material, such as a ferrous alloy of

chrome and nickel, or of chrome and manganese, but such alloys are far too expensive to be employed for the usual purposes of steel or wrought iron pipe. I therefore contemplate a process by which it is possible to form a thin protective alloy on the surface of a base metal such as a ferrous metal, although my invention, in its broader aspect, is not limited to the formation of an alloy, but generally contemplates providing a thin impervious and firmly anchored protective case for an article such as an iron or steel pipe.

In the drawing accompanying and forming a part hereof I have shown apparatus capable of being employed in carrying out my invention in connection with metal piping. Figure 1 is a side elevation of apparatus embodying my invention, portions being shown as broken away for convenience of illustration. Figure 2 is a transverse view of the apparatus shown in Figure 1, portions being shown in section for convenience of illustration. Figure 3 is a sectional end view taken on the lines III—III of Figure 1.

The apparatus illustrated is particularly adapted for applying a protective coating to metallic piping and I will therefore describe my invention as specifically applied to the coating of metallic piping.

During the operation of manufacturing iron or steel piping, the billet, after being pierced, is generally subjected to a reeling operation and/or an elongating operation wherein the pipe, while at a working temperature, is subjected to the working effect of rolls which engage its external surface.

In the drawing, I have illustrated one step of a pipe forming operation which happens to be a wall reducing operation. The pipe blank 4 encloses a mandrel 5, which is of less diameter than the internal diameter of the blank and which is free to move with the blank. The external surface of the blank is operated upon by oppositely disposed rolls 6 which rotate in the same direction and which cooperate with the mandrel 5 in such a way as to constitute the mandrel an idler working roll. It will be understood that the rolls 6 are crossed as shown in Figure 1 and are driven by any suitable means. Under such conditions the blank is not only rotated by the action of the roll 6 but is also moved forwardly in the direction of the horizontal arrow shown in Figure 1.

Guide rolls or disks 7 are employed in the particular reducing procedure illustrated. The axes of these rolls extend at right angles to the axis of the blank 4 or to the direction of longitudinal travel of the blank. These disks are so

located that they take the place of the ordinary stationary guides and are driven at a peripheral speed considerably higher than the longitudinal motion of the blank 4. As indicated by the arrows associated with these disks in the drawing, the disks are driven in the same direction and in such a direction as to give some propelling effect to the blank in the direction of its longitudinal travel. Each disk is grooved, as shown, so that its blank engaging surface substantially conforms to the contour of the pipe blank, although the disks are so located as to allow a small clearance between the inside of the blank 4 and the mandrel 5, as shown in Figure 2.

In the manufacture of wrought iron pipe it has been found that the guide disks should be driven at such a rate as to give them a peripheral speed much greater than the longitudinal speed of the blank, and this velocity ratio may be as great as one hundred to one in order to obtain or insure a substantially frictionless effect insofar as the rotative movement of the blank is concerned. When dealing with steel, a reduced ratio of velocities may be employed. It will be apparent that under the conditions described, the disks 7 do not change the wall thickness of the blank. They, however, do transform the peripheral elongation of the blank walls into a longitudinal elongation and have a decided burnishing action on the external surface of the blank. Under the speed and power conditions encountered, a tremendous amount of heat is generated at the point of contact between the disks and the blank, and conditions may be so controlled that sufficient heat will be generated to actually produce a molten film or skin on the surface of the blank.

I take advantage of this and also of the fact that the disks 7 explore every portion of the blank passing between them, by employing the disks as spreaders for the coating material. This material is therefore introduced onto the surface of the pipe blank immediately before the surface is engaged by the rapidly rotating disk and is preferably introduced in finely divided form and at a relatively high temperature.

It will be apparent that the coating material must have a melting or alloying temperature below the temperature of the tube but a vaporizing temperature above that temperature in order to be most effectively employed. For example, aluminum or copper dust may be blown onto the tube by pressure nozzles 8, one of which is shown located with its delivery aperture immediately adjacent one of the rolls 7 and so directed as to deposit a thin film of dust on the surface of the tube immediately prior to the time that surface is engaged by the adjacent disk 7. Under such conditions and particularly under the condition referred to, wherein the disks are driven at such a speed as to generate sufficient heat to produce a thin film or skin of molten metal at the surface of the blank, the coating material will not only be spread over the surface of the blank but will form an amalgam therewith, thus producing an atomic bond between the protective coating and the base metal.

By base metal I mean the metal of the blank and I employ the term throughout this specification merely to distinguish between the metal of the blank and the coating material. It will also be apparent that alloying material such as manganese, nickel and chromium may be delivered to the surface of the blank as above described.

While these materials may be delivered in pow-

dered form, it is preferable to deliver them in molten condition and to employ a spray nozzle 8 which is capable of delivering a thin film of molten metal to the surface of the blank at the points indicated in Figures 1 and 2. Where alloying metals are thus delivered the conditions must be such as to maintain the surface of the blank at an alloying temperature and this, as previously stated, can be accomplished by controlling the speed of the disks 7, it being understood that the blank is, under ordinary conditions, maintained at a working temperature, such as is usually employed in pipe piercing and pipe forming operations.

It will be understood that apparatus similar to that employed in spraying molten metal may be utilized in place of the nozzle 8 illustrated, and that the metal delivered may in itself be an alloy having a relatively high percentage of the alloying material, such as chromium, manganese or nickel, since the alloy so delivered will be somewhat diluted by the molten film or skin formed on the blank.

It will be apparent that the protective coating need not necessarily be composed of such material as will form an amalgam or an alloy with the base metal, since the conditions are such that a mechanical bond or an embedment may be relied upon. I therefore also contemplate employing protective materials having a melting point below the encountered temperatures of the blank and a vaporizing temperature above those temperatures, but such as will not form a chemical or atomic bond with the base metal. Under such conditions the disks 7 will not only accomplish the function of spreading the thin film of protective material over the surface of the blank but will also insure an embedment of the film, or the material of which the film is composed, in the surface of the blank but will also insure a uniformity of the film. That is to say, the action of the disks in connection with the alloying or non-alloying material will be such as to insure the spreading of an impervious coating over the surface of the blank provided, of course, sufficient coating material is delivered to form an impervious and uniform cover.

From the foregoing it is apparent that a protective coating may be firmly secured or anchored to the surface of a base metal, without greatly increasing the cost of the article being manufactured. For example, an alloy, as above described, approximately .003 inch thick, may be formed on the surface of a 24 inch O. D. x 1/4 inch wall pipe, 35 feet long and weighing a gross ton, by utilizing approximately four pounds of chromium and two and one-half pounds of nickel in the production of a surface alloy having 18 percent chromium and 8 percent nickel. While the cost of producing such a surface is relatively low, the pipe so coated will resist external corrosion as effectively as if the entire pipe were made from the non-corrosive alloy. It will also be apparent that the coating operation adapts itself to the use of different alloying materials so that the alloy may be selected in accordance with the conditions encountered in service, and that the vehicle employed for delivering the coating material to the surface of article coated is more or less unimportant so long as it is capable of delivering a thin film of either powdered or molten material to the surface.

It will be apparent that while I have illustrated and described my process in connection with apparatus employing rapidly rotating disks as well

as the working rolls 6, the process may be carried forward in connection with any form of rotating spreading rolls. That is to say, the finely divided coating material, whether powdered or molten, 5 may be delivered to the surface of the blank immediately adjacent the working rolls operating on the blank, and particularly where the pressures encountered and the speed of operation is such that the effect of the working rolls is to impart 10 heat to the blank.

It is also apparent that while I have illustrated the invention in connection with pipe forming machinery that the invention is not so limited and that various changes, additions, omissions 15 and modifications may be made in the procedure contemplated, and various substitutions of material may be resorted to, without departing from the spirit and scope of the invention as set forth by the appended claims.

20 I claim:

1. The method of forming a protective coating on the surface of a base metal which consists in delivering a thin film of coating material to a portion of such surface while maintaining such 25 portion at least at a forging temperature, and then in subjecting the base metal and the coating material to a burnishing action of a magnitude sufficient to generate heat of sufficient quantity to form a molten film of the base metal and 30 coating material.

2. The method of forming a protective coating on the surface of a base metal which consists in delivering a thin film of alloying metal to a portion of such surface while maintaining such portion at least above the alloying temperature of 35 said alloying metal, and then in raising the temperature of such portion of the surface by subjecting the base metal and alloying metal to a burnishing action of sufficient magnitude to generate heat of sufficient quantity to form a molten film of the base metal and alloying metal.

40 3. The method of forming a fine protective coating on the surface of a base metal which consists in delivering a thin film of alloying material

to a portion of such surface while maintaining such portion at least above the alloying temperature of said alloying material and then in helically working said base metal while subjecting the same and the alloying material to a burnishing action of sufficient magnitude to generate heat of sufficient quantity to form a molten film 5 of the base metal and alloying material.

4. The method of forming a protective coating on the surface of a base metal which consists in delivering a thin film of alloying metal to a portion of such surface while maintaining such portion at least above the alloying temperature of said alloying metal, and then in raising the temperature of such portion of the surface by 10 subjecting the base metal and said alloying metal to a helical burnishing action of sufficient magnitude to form a molten film of the base metal and the alloying metal.

5. The method of forming a fine protective 20 coating on the surface of a base metal which consists in delivering a thin film of alloying metal to a portion of such surface while maintaining such portion at least above the alloying temperature of said alloying metal, then in subjecting the 25 base metal and the alloying metal to a burnishing action in order to generate heat of sufficient quantity to form a molten alloy film of base metal and alloying metal, and finally in helically working the molten film to form a complete protective 30 coating.

6. The method of forming a protective coating on the surface of a base metal which consists in delivering a thin film of coating material to a portion of such surface while maintaining such 35 portion at least at a forging temperature, then in subjecting the base metal and the coating material to a burnishing action of a magnitude sufficient to generate heat of sufficient quantity to at least melt the coating material, and subsequently 40 working and helically spreading the melted coating material to form a continuous coating on the surface of the base metal.

BRYANT BANNISTER.